

## UNITED STATES PATENT OFFICE

2,511,746

## ANTIOXIDANTS FOR MINERAL OIL LUBRICANTS AND COMPOSITIONS CONTAINING THE SAME

Herschel G. Smith, Wallingford, and Troy L. Cantrell, Lansdowne, Pa., and John G. Peters, Audubon, N. J., assignors to Gulf Oil Corporation, Pittsburgh, Pa., a corporation of Pennsylvania

No Drawing. Application December 8, 1948,  
Serial No. 64,238

16 Claims. (Cl. 252—50)

**1**  
This invention relates to antioxidants for mineral oil lubricants and compositions containing the same, and more particularly, it relates to addition agents for mineral oil lubricants which inhibit the oxidative deterioration of said lubricants.

In the lubrication of internal combustion engines of all types, particularly when severe operating conditions are encountered, plain mineral lubricating oils often prove unsatisfactory in service because of the oxidative deterioration of the oil, with the attendant deposition on the engine surfaces of varnish, gum or sludge. Furthermore, many lubricating oil compositions which may be highly satisfactory for the lubrication of other mechanisms have been found wholly unsuitable for use as turbine oils.

The formation of varnishes, gums and sludges on engine surfaces is due at least in part to oxidation effects on mineral lubricating oils. In turbine oils the problem of oxidation is further aggravated, because in normal use turbine oils rapidly become contaminated with water.

It is an object of this invention, therefore, to provide an addition agent for mineral oil lubricants which will inhibit the oxidative deterioration of such lubricants.

It is a further object of this invention to provide improved mineral oil lubricant compositions which are remarkably stable against oxidation under service conditions.

These and other objects are accomplished by the present invention wherein an addition agent for mineral oil lubricants is prepared by condensing N-amyylaniline, N-dimethylaniline and formaldehyde in the presence of an activated clay catalyst, and recovering the condensation product. The condensation product so obtained is a light-colored product which, when added to mineral oil lubricants, confers a remarkably stability against deterioration by oxidation. Such condensation products and the mineral oil lubricant compositions containing them are believed to be novel and are considered parts of our invention. Contrary to what may be expected from the nature of the reactants, we do not obtain highly condensed, insoluble resinous products. On the contrary, when the above reactants are condensed in accordance with our invention, there are obtained light-colored condensation products which are non-resinous and which are readily soluble in mineral oils.

In performing the condensation, the reactants are mixed and heated to a maximum temperature of 350° F. We have found that if the tempera-

**2**  
ture of 350° F. is exceeded to any substantial extent, the condensation product formed tends to be resinous and insoluble. In general, the preferred temperature for the condensation ranges from 150° to 300° F.

The proportions of the reactants vary over a fairly wide range. For each mol of N-amyylaniline, there is employed from 1 to 4 mols of N-dimethylaniline and from 1 to 4 mols of formaldehyde. Ordinarily, it is preferred to use from 5 to 10 per cent by weight of the activated clay catalyst, based on the total weight of the reactants. However, smaller amounts, as low as 1 per cent by weight, and larger amounts, as high as 20 per cent by weight, may also be employed; but larger amounts than about 10 per cent by weight are ordinarily not necessary.

In lieu of formaldehyde, and formaldehyde-yielding compound, such as paraformaldehyde, dioxymethylene and trioxymethylene may be employed. In such case, the amount of formaldehyde-yielding compound used is based on the equivalent number of mols of formaldehyde yielded within the range of proportions of formaldehyde set forth hereinabove. Accordingly, as used in the appended claims, the term "formaldehyde" is intended to include formaldehyde-yielding compounds as well as formaldehyde itself.

**30** Various activated clay catalysts may be employed in accordance with our invention. Such materials are well known in the art and comprise a natural clay, such as bentonite, fuller's earth, florian and smectite, which has been acid treated in order to activate the clay. These materials are described in U. S. Patent 1,893,165, for example.

**40** In preparing our new addition agents, the reactants and catalyst are placed into a reaction vessel which is then closed and the mixture heated with agitation under reflux until all of the formaldehyde or formaldehyde-yielding compound has been consumed. At this time, the water which is formed as a result of the condensation is removed, preferably under vacuum, and the dehydrated condensation product is then filtered to remove the activated clay catalyst. In some instances, it is desirable to prepare our new addition agent in a concentrate in a mineral lubricating oil which may then be diluted down with additional oil to the concentration desired in the final lubricating composition. In such instances, the mineral lubricating oil may be added in a suitable amount, say in a weight equal to the weight of reactants, to the reaction mix-

ture in the reaction vessel, and the condensation product obtained will then be a concentrated solution of the addition agent in the mineral lubricating oil.

The condensation products obtained in accordance with our invention are liquids or crystalline solids. While the exact nature of the chemical composition of the condensation products is unknown, all of the three reactants enter into a final unitary product. The exact manner in which the catalyst influences the reaction is unknown. However, regardless of any theory involved, the use of an activated clay catalyst is an essential feature of our invention, since if the catalyst is omitted, black, insoluble, resinous condensation products are obtained.

The following examples illustrate the preparation of our new addition agent:

*Example I.*—Into an iron vessel, there was introduced 1 pound mol of N-amyylaniline (163 pounds), 4 mols of N-dimethylaniline (484 pounds) and 4 mols of formaldehyde in a 37 per cent by weight aqueous solution (320 pounds). To this mixture, there was added 62 pounds of Filtrol (an activated montmorillonite catalyst). The vessel was closed and attached to a reflux condenser. The mixture was then heated to 210° F. and refluxed for 12 hours. The condensation product was then dried by distilling off all water, both that added with the formaldehyde and formed in the reaction, by heating at 290° F. The product was then filtered. It had the following properties:

|                    |     |    |          |              |
|--------------------|-----|----|----------|--------------|
| Gravity, °A. P. I. | 5.7 | 35 | Base Oil | Improved Oil |
| Color, N. P. A.    | 2.5 |    |          |              |
| Neutralization No. | 0.9 |    |          |              |

*Example II.*—Example I was repeated using 1 mol of N-amyylaniline, 3 mols of N-dimethylaniline, 3 mols of formaldehyde and about 3 per cent by weight of an activated clay. The filtered product had the following properties:

|                    |     |    |          |              |
|--------------------|-----|----|----------|--------------|
| Gravity, °A. P. I. | 6.8 | 45 | Base Oil | Improved Oil |
| Color, N. P. A.    | 2.5 |    |          |              |
| Neutralization No. | 1.0 |    |          |              |

*Example III.*—Another antioxidant was prepared under the conditions outlined in Example I using 1 mol of N-amyylaniline, 3 mols of N-dimethylaniline, 4 mols of formaldehyde and 15 per cent by weight of Filtrol (activated montmorillonite). The filtered product had the following properties:

|                    |     |    |          |              |
|--------------------|-----|----|----------|--------------|
| Gravity, °A. P. I. | 4.0 | 55 | Base Oil | Improved Oil |
| Color, N. P. A.    | 3.0 |    |          |              |
| Neutralization No. | 1.8 |    |          |              |

The N-amyylaniline used in the above examples was the normal amyl isomer. However any of the isomeric N-amyylanilines may be used with good results.

The condensation products obtained in accordance with the above disclosure from N-amyylaniline, N-dimethylaniline and formaldehyde in the presence of an activated clay catalyst are excellent addition agents for mineral oil lubricants. They are readily soluble in all types of mineral oils, that is paraffinic, naphthenic or mixed base mineral oils and can be blended with mineral oils in high proportions to form concentrated solutions thereof, which may then be diluted down to the proportions desired in the final mineral oil lubricant composition. As stated, our new addition agents are remarkably effective in inhibiting the oxidative deterioration of mineral oil lubricant compositions. For this purpose

small amounts of our new addition agents are generally sufficient. For example, our addition agents may be added to mineral lubricating oils in minor amounts, say from 0.001 to 1 per cent by weight on the mineral oil, sufficient to inhibit the oxidative deterioration of the oil. Larger amounts of our new addition agents may be used if desired but it is ordinarily unnecessary to do so.

The following examples illustrate the remarkable antioxidant effects of our new addition agents. In the following examples, the base oil and the same oil blended with our new addition agents are subjected to a standard oxidation test which measures the stability of the oils to oxidation. The oxidation test referred to is a standard test designated ASTM D943-47 T. Briefly, the test comprises subjecting the oil sample to oxygen at a temperature of 95° C. (203° F.) in the presence of water and an iron-copper catalyst, and determining the time required to build up a neutralization number of 2. The flow of oxygen is maintained at 3 liters per hour. The remarkably effective stability to oxidation of mineral oil lubricant compositions containing our new addition agents is illustrated by the results shown in the following examples.

*Example IV.*—An improved steam turbine oil was prepared by treating a turbine oil base stock with 0.5 per cent by weight of an additive prepared according to Example I. A comparison of the properties of the base oil and improved turbine oil showed the following:

|                                             | Base Oil | Improved Oil |
|---------------------------------------------|----------|--------------|
| Gravity, °API                               | 28.6     | 28.4         |
| Oxidation Test, ASTM D943-47T 203° F., 3 L. |          |              |
| Oxygen per Hr.                              | 180      | 4,210        |
| Time Oxidized, Hrs.                         | 2.0      | 2.0          |
| Neutralization No.                          |          |              |

*Example V.*—An improved motor lubricating oil was prepared by treating a highly refined motor lubricating oil base stock with 0.5 per cent by weight of the antioxidant prepared according to Example I. A comparison of the properties of the base oil and the improved oil showed:

|                                             | Base Oil | Improved Oil |
|---------------------------------------------|----------|--------------|
| Gravity, °API                               | 30.5     | 30.1         |
| Viscosity, S.U.V. 210° F.                   | 75.5     | 74.2         |
| Color, N.P.A.                               | 2.75     | 2.75         |
| Oxidation Test, ASTM D943-47T 203° F., 3 L. |          |              |
| Oxygen per Hr.                              | 210      | 4,020        |
| Time Oxidized, Hrs.                         | 2.0      | 2.0          |
| Neutralization No.                          |          |              |

The above examples show the remarkable oxidation stability imparted to mineral oil lubricant compositions by the use of our new addition agents. Mineral oil lubricant compositions containing our new addition agents are therefore eminently suited for use where the operating conditions are extremely severe, as in Diesel, tank and truck engines, and in the lubrication of steam turbines.

The notable effects of our new addition agents cannot be readily accounted for and cannot be predicted from the nature of the reactants. Thus, condensation products prepared from other functionally similar compounds have been found to be either prooxidant or to show no antioxidant effects whatsoever. For example, we have prepared condensation products similar to our new addition agents by substituting xylidine for the N-dimethylaniline. The resulting condens-

sation products were found to be entirely unsuitable for inhibiting the oxidative deterioration of mineral oil lubricant compositions.

While we have shown in the examples the preparation of compounded lubricating oils, our invention is not limited thereto but comprises all mineral oil lubricant compositions containing our new addition agents, such as greases and the like. If desired, other known addition agents may be incorporated into the lubricant compositions prepared in accordance with our invention. For example, pour point depressants, extreme-pressure agents, viscosity index improvers and the like may be added.

Resort may be had to such modifications and variations as fall within the spirit of the invention and the scope of the appended claims.

We claim:

1. The process of preparing an addition agent for mineral oil lubricants which comprises heating 1 mol of N-amyylaniline, 1 to 4 mols of N-dimethylaniline, and 1 to 4 mols of formaldehyde in the presence of an activated clay catalyst at a temperature not in excess of 350° F. to condense together the three reactants, and recovering the condensation product.

2. The process of preparing an addition agent for mineral oil lubricants which comprises heating 1 mol of N-amyylaniline, 1 to 4 mols of N-dimethylaniline, and 1 to 4 mols of formaldehyde in the presence of an activated clay catalyst at a temperature of from 150° to 300° F. to condense together the three reactants, and recovering the condensation product.

3. The process of preparing an addition agent for mineral oil lubricants which comprises adding 1 mol of N-amyylaniline, 1 to 4 mols of N-dimethylaniline, 1 to 4 mols of formaldehyde and from 5 to 10 per cent by weight on the foregoing reactants of an activated clay catalyst to a mineral lubricating oil, heating the mixture at a temperature of from 150° to 300° F. to condense together the three reactants, and recovering a solution of the condensation product in the mineral lubricating oil.

4. The process of preparing an addition agent for mineral oil lubricants which comprises heating 1 mol of N-amyylaniline, 4 mols of N-dimethylaniline and 4 mols of formaldehyde in the presence of 5 to 10 per cent by weight of an activated clay catalyst at a temperature of from 150° to 300° F. to condense together the three reactants, and recovering the condensation product.

5. The process of preparing an addition agent for mineral oil lubricants which comprises heating 1 mol of N-amyylaniline, 3 mols of N-dimethylaniline and 3 mols of formaldehyde in the presence of 5 to 10 per cent by weight of an activated clay catalyst at a temperature of from 150° to 300° F. to condense together the three reactants, and recovering the condensation product.

6. The process of preparing an addition agent for mineral oil lubricants which comprises heating 1 mol of N-amyylaniline, 3 mols of N-dimethylaniline and 4 mols of formaldehyde in the presence of 5 to 10 per cent by weight of an activated clay catalyst at a temperature of from 150° to 300° F. to condense together the three reactants, and recovering the condensation product.

7. A non-resinous condensation product of 1 mol of N-amyylaniline, 1 to 4 mols of N-dimethylaniline and 1 to 4 mols of formaldehyde, said

product being obtained by the process of claim 1.

8. A non-resinous condensation product of 1 mol of N-amyylaniline, 4 mols of N-dimethylaniline and 4 mols of formaldehyde, said product being obtained by the process of claim 4.

9. A non-resinous condensation product of 1 mol of N-amyylaniline, 3 mols of N-dimethylaniline and 3 mols of formaldehyde, said product being obtained by the process of claim 5.

10. A non-resinous condensation product of 1 mole of N-amyylaniline, 3 mols of N-dimethylaniline and 4 mols of formaldehyde, said product being obtained by the process of claim 6.

11. A lubricant composition comprising a major amount of a mineral lubricating oil, and a minor amount, sufficient to inhibit the oxidative deterioration of said oil of a non-resinous condensation product of 1 mol of N-amyylaniline, 1 to 4 mols of N-dimethylaniline and 1 to 4 mols of formaldehyde, said product being obtained by the process of claim 1.

12. A lubricant composition comprising a major amount of a mineral lubricating oil, and a minor amount, from 0.001 to 1.0 per cent by weight of said oil, of a non-resinous condensation product of 1 mol of N-amyylaniline, 1 to 4 mols of N-dimethylaniline, and 1 to 4 mols of formaldehyde, said product being obtained by the process of claim 1.

13. A lubricant composition comprising a major amount of a mineral lubricating oil, and a minor amount, sufficient to inhibit the oxidative deterioration of said oil, of a non-resinous condensation product of 1 mol of N-amyylaniline, 4 mols of N-dimethylaniline, and 4 mols of formaldehyde, said product being obtained by the process of claim 4.

14. The composition of claim 16, wherein said condensation product is present in an amount of 0.5 per cent by weight.

15. A lubricant composition comprising a major amount of a mineral lubricating oil, and a minor amount, sufficient to inhibit the oxidative deterioration of said oil, of a non-resinous condensation product of 1 mol of N-amyylaniline, 3 mols of N-dimethylaniline and 3 mols of formaldehyde, said product being obtained by the process of claim 5.

16. A lubricant composition comprising a major amount of a mineral lubricating oil, and a minor amount, sufficient to inhibit the oxidative deterioration of said oil, of a non-resinous condensation product of 1 mol of N-amyylaniline, 3 mols of N-dimethylaniline and 4 mols of formaldehyde, said product being obtained by the process of claim 6.

HERSCHEL G. SMITH.

TROY L. CANTRELL.

JOHN G. PETERS.

#### REFERENCES CITED

The following references are of record in the file of this patent:

#### UNITED STATES PATENTS

| Number    | Name     | Date          |
|-----------|----------|---------------|
| 1,584,473 | Regal    | May 11, 1926  |
| 1,954,484 | Mattison | Apr. 10, 1934 |

#### FOREIGN PATENTS

| Number  | Country       | Date          |
|---------|---------------|---------------|
| 12,021  | Australia     | Feb. 29, 1926 |
| 256,394 | Great Britain | Aug. 12, 1926 |
| 264,958 | Italy         | Mar. 18, 1929 |

**Certificate of Correction**

Patent No. 2,511,746

June 13, 195

HERSCHEL G. SMITH ET AL.

It is hereby certified that errors appear in the printed specification of the above numbered patent requiring correction as follows:

Column 1, line 40, for the word "remarkably" read *remarkable*; column 2, line 18, for "and" read *any*; column 6, line 39, for the claim reference numeral "16" read *18*;

and that the said Letters Patent should be read with these corrections therein that the same may conform to the record of the case in the Patent Office.

Signed and sealed this 5th day of September, A. D. 1950.

[SEAL]

THOMAS F. MURPHY,  
*Assistant Commissioner of Patents.*